

Feb. 14, 1956

D. W. LIGHT

2,734,532

LAMINATED PAPER YARNS AND FABRICS, INCLUDING THE SAME

Filed July 31, 1951



# United States Patent Office

2,734,532

Patented Feb. 14, 1956

1

2,734,532

## LAMINATED PAPER YARNS AND FABRICS INCLUDING THE SAME

Donald W. Light, Wayland, Mass.

Application July 31, 1951, Serial No. 239,518

2 Claims. (Cl. 139—420)

The present invention relates to yarns to be used particularly as weft and stuffer warp yarns for carpets and similar fabrics, but can also be used to advantage in other weaving, serving, and stuffing or spacing applications. Although less expensive than the textile and bast fibre yarns they replace, the acceptance of the paper yarns heretofore available for use in carpets and other applications has been slow due to their low strength, stiffness or wiriness, tendency to kink or twist, and slipperiness.

Heretofore such yarns have been made by slitting paper into ribbons that simulate textile fibre slivers and twisting these into a yarn, following closely the traditional methods and using the same type of equipment as in the textile industry. In the attempt to adapt paper to this process and at the same time alleviate the serious objections enumerated above, much experimenting has been done and some improvements have been effected, but the basic faults remain. So far as I know there has been no attempt to develop a process and a yarn designed around and taking advantage of the inherent characteristics of paper rather than trying to adapt it to the established textile-yarn processes.

The present invention utilizes the wide widths in which paper is produced, for I have discovered that a more satisfactory yarn can be made by laminating plies of suitable paper with a flexible adhesive and then slitting the wide paper mass into strips whose width is preferably about equal to the thickness of the laminated sheet so that preferably the yarn has a square cross-section. My present invention also includes the novel fabric made with such yarn. My invention also includes fabrics and particularly carpets in which some of the yarns and particularly stuffer warps are or may be rectangular in cross section so that they take the place of two or more twisted yarns laid side by side.

The invention will be readily understood from the following description taken in conjunction with the accompanying drawings in which:

Fig. 1 is a diagrammatic view of a machine by which the yarn may be produced.

Fig. 2 is a section on line 2—2 of Fig. 1 after slitting.

Fig. 3 is a yarn greatly exaggerated in size to illustrate its construction.

Fig. 4 is a yarn having somewhat different dimensions.

Fig. 5 is a section of a piece of carpet in which the yarn embodying the invention is employed as a weft.

Fig. 6 is a section of another carpet in which a yarn of essentially square cross section is used as a weft; and

Fig. 7 is a section of the carpet shown in Fig. 6 and taken at right angles, yarn of rectangular cross section embodying my invention being used as a stuffer warp in place of two or more twisted yarns ordinarily used.

Referring now to the drawings and particularly to Fig. 1, webs of paper 11 are withdrawn from rolls 12, coated with a flexible adhesive as indicated at 13, then brought together and pressed between rollers 14 and then passed over drums 15 that are heated if emulsion type adhesive is used and requires drying, or that are cooled if a hot

2

melt adhesive is used. Thereafter the laminated sheet A is passed through a slitter 16 and the yarns B thus formed are wound on a beam 17 from which they may be withdrawn during weaving rewinding or during whatever other operation that is required. For convenience the drawings illustrate a laminate containing only six plies of paper, but it is readily apparent that the arrangement is adaptable to any desired number of plies, the number of which will be dependent upon the thickness of yarn desired and 10 the weight or thickness of the paper constituting the plies. There are, of course, numerous variations possible in the arrangement of the devices coating the layers and laminating them, but it is believed that Fig. 1 clearly illustrates the basic steps and the principles involved. Fig. 1 shows 15 a continuous production of yarn from a web, but it is evident that such production can be split up into a number of separate operations if desired. The heavy laminated sheet A can be built up by several separate laminating operations; and the slitting can be done separately or can be done by stages. Any machine or procedure 20 may be adopted which will superpose several plies of paper, secure them together, and cut strands therefrom.

The laminated sheet A produced by the machine shown in Fig. 1 is shown in Fig. 2 and the slits separating the 25 sheet into yarns B are spaced so that the width and thickness of the yarns B thus formed will be about equal and consequently the yarn will be about square in cross section as shown in Fig. 3. In Fig. 4 is shown a yarn which is wider than its thickness and is useful particularly for 30 stuffer warps in carpets where the stuffing or spacing characteristics are more important than the yarn's flexibility. More than one ordinary textile or twisted yarn may be replaced thereby.

As shown in the drawings, the thickness of the yarns 35 B at least approximate their width so that the yarns have substantial thickness in comparison with their width. The yarns B are thus of suitable body and dimension to replace conventional filler or stuffer yarns in fabrics such as carpets as opposed to strips of material which are thin 40 compared with their width and which are useful for plaiting mats and the like but are not suitable for stuffer yarns for fabrics such as carpets.

In the manufacture of yarn embodying the invention 45 various types of paper can be used but I employ preferably a high quality kraft paper of maximum fibre orientation and strength in the machine direction. Aside from a high machine direction tensile strength such a paper is generally characterized by a higher ratio of cross direction to machine direction tear, greater porosity, and lower 50 density than the usual kraft paper. Kraft paper of almost any weight up to one hundred and fifty pounds per ream might be used but I prefer paper within the range of twenty-five to sixty pounds per ream, and more particularly about forty pounds per ream.

One advantage of the present invention is that it can 55 make use of the more economical heavier weight papers that are not adaptable for twisting into finer gauge yarns because of the limitation of handling the narrower widths of ribbons entailed. Where yarn with high wet strength is required, high wet strength paper may be employed, for instance, treated with melamine-formaldehyde, urea-formaldehyde, or other suitable resins well known to the paper making art.

The adhesive employed may be either an emulsion or 60 dispersed type or a hot melt. It must provide a good bond and be flexible as contrasted with the thermosetting resin adhesives used in conventional paper laminates of comparable thickness for panels in the building, decorative, and electrical industries. The adhesive should also be water resistant. Rubber base adhesives are satisfactory, as are adhesives based upon synthetic elastomers or 65 plasticized copolymer resins, e. g., polyvinyl acetate emul-

sion compounded with dibutyl phthalate plasticizer. In fact, asphalt adhesives modified with rubber or synthetic copolymers to improve flexibility are satisfactory where the color and solvent susceptibility of the asphalt are not objectionable. It is desirable that lamination of the paper webs with any of these adhesives be accomplished with a minimum of saturation of the paper by the adhesive in order to obtain maximum flexibility.

The flexibility of the adhesive and the bond has a direct bearing on not only the yarn's flexibility but also upon its knot or "cut" strength. When folded or knotted the plies will conform or adjust at areas of high stress when a flexible adhesive is used, whereas with conventional inflexible adhesives the plies will shear and the yarn will have poor strength when distorted.

A satisfactory yarn is made with twelve plies of twenty-five pounds per ream kraft paper and a rubber latex base adhesive. This yarn had an average thickness of about .031 inch and was slit to have a width of .03 inch. The yarn measured about eight hundred and forty yards per pound.

When such a yarn is used for the weft H of a woven fabric, such as that indicated in Figs. 5 and 6, it will be found to be particularly satisfactory since the other threads and yarns pressed against it in the woven structure, tend to indent or form depressions in the edges of the square laminated yarn with the result that abnormal slippage between yarns is eliminated and the whole fabric structure is stabilized. Such weft yarns have good strength and wearing qualities and sufficient bulk to give a full plump appearance to the fabric. In Fig. 7 I have shown

how a single stuffer warp G of rectangular cross section may be used in place of two or more twisted stuffer warp yarns. It will be understood that the particular uses of the yarns embodying my invention shown in the drawings and foregoing description are merely by way of illustration, since the yarn is capable of many other uses.

I claim:

1. A woven fabric comprising a warp of conventional fibre yarn, a weft including untwisted yarn of quadrilateral cross-section having sharp corner edges and flat sides, said untwisted yarn being composed exclusively of several superposed layers of paper secured to each other solely by a flexible adhesive and said warp being drawn across the said sharp corner edges of the weft.
2. A woven fabric comprising a warp and a weft and including conventional fibre yarns and untwisted yarns of quadrilateral cross-section having sharp corner edges and flat sides, said untwisted yarns being composed of several superposed layers of paper secured to each other solely by a flexible adhesive and said conventional fibre yarns being drawn across said sharp edges of said untwisted yarns.

References Cited in the file of this patent

UNITED STATES PATENTS

|           |            |               |
|-----------|------------|---------------|
| 1,810,438 | Rado       | June 16, 1931 |
| 1,829,299 | Rosenstein | Oct. 27, 1931 |
| 1,852,451 | Everett    | Apr. 5, 1932  |
| 1,913,397 | Knecht     | June 13, 1933 |
| 2,492,670 | Underwood  | Dec. 27, 1949 |